# EUROPEAN PATENT SPECIFICATION

(11) **EP 0 369 822 B1**
(45) Date of publication and mention of the grant of the patent: **30.12.1992**
(21) Application number: 89311957.8
(22) Date of filing: 17.11.1989
(51) Int. Cl.: D04B 1/18

(54) **Knitted stretch lace**
Gestrickte elastische Spitze
Dentelle élastique tricotée

(30) Priority: 17.11.1988 GB 8826908
(43) Date of publication of application: 23.05.1990
(73) Proprietor: CHATSWORTH KNITTING LIMITED, Bagworth Leicestershire LE6 1BH (GB)
(72) Inventor: Collins, Michael Charles, Nr Melton Mowbray Leicestershire (GB); Shaw, Ronald Arthur, New Wessington Derbyshire (GB); Farmer, Geoffrey Raymond, Atherstone Warwickshire (GB)
(74) Representative: Ablewhite, Alan James

(56) References cited:
- FR-A- 1 111 695
- FR-A- 1 464 865
- GB-A- 765 882
- GB-A- 1 507 973
- US-A- 4 062 204

## Description

This invention relates to a knitted fabric having the visual effect of lace, but having stretch and recover characteristics, as already known from GB-A 765 882.

True laces, eg Raschel or Leavers laces, are made on lace machines and are generally adapted to provide narrow piece goods, for example edgings and trimmings. Lace of this type can be made in a stretch and recover form, using an elastane such as Lycra (Trade Mark). There is, however. a requirement for wide piece goods in the form of patterned lace, or more accurately lace-type knitted fabric, which exhibits good stretch and recover characteristics and thus lends itself to use in bodywear and intimate apparel such as leotards, tights etc. However, heavy lace effects carrying a dense pattern (e.g. of the guipure type) are difficult to produce when they contain a pattern of staple fibre, especially in wide pieces, since modern lace machinery is generally adapted to deal with extruded filament-based yarn.

We have now devised a method of producing a stretch and recover lace-type fabric on a double, or single jersey knitting machine, by knitting a ground of a combination of contractile and non-contractile yarn together with a pattern of staple or other yarn and then heat setting the fabric to stabilise the contractile yarn.

According to the invention we provide a stretchable knitted fabric having the visual effect of lace, comprising a ground of monofil synthetic filament co-knitted with a contractile yarn, and a pattern provided by a third co-knitted yarn, the knitted fabric having been preset at a temperature of from 185 to 205°C. In general, the ground is produce of a combination of an elastane such as Lycra, Dorlaston, Spandex (Registered Trade Marks) etc, and a monofil synthetic filament, e.g. a polyamide or polyester. In view of the temperature used in the heat setting, a polyamide such as nylon 66 is most preferred. The monofil filament is preferably from 10 to 45 dtex.

The elastane may be a "bare" elastane, or a covered yarn in which the elastane is wound with a second fibre, generally a polyamide, although cotton or another cellulosic fibre, or polyesters, or mixtures thereof can be used. In a preferred embodiment, the elastane is covered with a polyamide of from 33 to 78 dtex. While all yarn run to the knitting machine must be under a suitable tension, it is important that the elastane is under suitable tension, which in turn depends on the degree of stretch and stretch recovery required in the finished product. Typically for an elastane of from 33 to 156 dtex a tension of 2-4grms per end is suitable.

The monofil and the elastane are knitted together on the same needles, preferably on a yarn-for-yarn basis, although the yarn proportion can vary from 1:1 as required.

The amount of the third yarn used for the pattern effect will, of course, depend on the amount of patterning provided. Typically the pattern yarn is a staple fibre, in particular a cellulosic fibre such as cotton or a synthetic such as rayon. Where a staple cotton yarn is used, a cotton count of about 1/8's to 1/60's, e.g. 1/22's or 1/30's, is suitable, depending on the machine gauge. Cellulose-based pattern yarns are preferred, partly because of suitability for the heat treatment, and also for the ease of dyeing, but primarily for the aesthetic appeal. In a preferred embodiment the fabric comprises a ground of polyamide monofil and polyamide-covered elastane and a pattern of cotton staple.

The fabric is knitted on a conventional jersey machine, especially a double jersey weft knitting machine, e.g. of gauge 8 to 32. Electronic jacquard machines are particularly suitable for detailed pattern work on a large area.

It is an important part of the process that the knitted fabric is heat set at a temperature of 185 to 205°C, preferably about 195°C, in order to prevent contraction of the elastane. In a typical procedure, a double jersey is slit open onto an A frame and heat set a 195°C at a speed of about 16m/min, preferably on an indirectly heated stenter. After this heat treatment, the fabric can be passed through one or more dying procedures, typically jet-dyeing the nylon content, drying at, say, 140 to 150°C, and then pad dyeing the cellulosic content, followed by a stenter softening process and drying.

By operating in this way, it is possible to produce a fine lace-effect knitted fabric which is smooth and un-gathered, but which has good stretch and recovery characteristics coupled with a pattern effect which can be produced in staple yarn.

## Claims

1. A stretchable knitted fabric having the visual effect of lace, characterised by a ground of monofil synthetic filament co-knitted on the same needles with a contractile yarn, and a pattern provided by a third co-knitted yarn, the knitted fabric having been pre-set at a temperature of from 185 to 205°C.

2. A knitted fabric according to claim 1, in which the third yarn forming the pattern is a staple yarn.

3. A knitted fabric according to claim 2, in which the staple yarn is a cellulosic yarn.

4. A knitted fabric according to any of claims 1 to 3, in which the contractile yarn comprises an elastane, either bare or covered with a second yarn.

5. A knitted fabric according to claim 4 in which the elastane is from 33 to 156 dtex.

6. A knitted fabric according to any of the proceeding claims in which the monofil is from 10 to 45 dtex.

7. A knitted fabric according to claim 4 or claim 5, in which the elastane is covered with a polyamide of from 33 to 78 dtex.

8. A knitted fabric according to any of claims 1 to 7 comprising a ground of polyamide monofil and polyamide-covered elastane and a pattern of cotton staple.

9. A process for the production of a stretchable knitted fabric having the visual effect of lace, characterised in knitting together monofil synthetic filament and a contractile yarn to form a ground and a third yarn to form a lace-type pattern and heat setting the knitted fabric at a temperature of from 185 to 205°C.

## Patentansprüche

1. Dehnbare gewirkte Maschenware, die die optische Wirkung von Spitze hat, gekennzeichnet durch ein Grundgewebe aus auf gleichen Nadeln mit einem zusammenziebaren Garn zusammengewirkter monofiler synthetischer Filamentfaser, und ein durch ein drittes zusammengewirktes Garn geliefertes Muster, wobei die gewirkte Maschenware bei einer Temperatur im Bereich von 185 bis 205°C vorfixiert worden ist.

2. Gewirkte Maschenware nach Anspruch 1, bei der das das Muster formende dritte Garn ein Stapelgarn ist.

3. Gewirkte Maschenware nach Anspruch 2, bei der das Stapelgarn ein Zellulosegarn ist.

4. Gewirkte Maschenware nach einem der Ansprüche 1 bis 3, bei der das zusammenziehbare Garn ein entweder nacktes oder mit einem zweiten Garn bedecktes Elastan enthält.

5. Gewirkte Maschenware nach Anspruch 4, bei der das Elastan zwischen 33 bis 156 dtex liegt.

6. Gewirkte Maschenware nach einem der vorhergehenden Ansprüche, bei der der monofile Faden zwischen 10 bis 45 dtex liegt.

7. Gewirkte Maschenware Anspruch 4 oder Anspruch 5, bei der das Elastan mit einem Polyamid von 33 bis 78 dtex bedeckt ist.

8. Gewirkte Maschenware nach einem der Ansprüche 1 bis 7, die ein Grundgewebe aus Polyamidmonofilfaden und polyamidbedecktem Elastan und ein Muster aus Baumwollstapel aufweist.

9. Verfahren zur Hersellung einer dehnbaren gewirkten Maschenware, die die optische Wirkung von Spitze hat, gekennzeichnet durch das Zusammenwirken monofilen synthetischen Filamentes und eines zusammenziehbaren Garns zur Bildung eines Grundgewebes und eines dritten Garns zur Bildung eines spitzenartigen Musters, und eine Wärmefixierung der gewirkten Maschenware bei einer Temperatur im Bereich von 185 bis 205°C.

## Revendications

1. Un tissu tricoté extensible ayant l'aspect de la dentelle, caractérisé par un fond de filament synthétique monofilaire tricoté ensemble, avec les mêmes aiguilles, avec un fil contractile, et par un dessin fourni par un troisième fil tricoté en même temps, le tissu tricoté ayant été préfixé à une température comprise entre 185 et 205°C.

2. Un tissu tricoté selon la revendication 1, dans lequel le troisième fil formant le dessin est un fil de fibres discontinues.

3. Un tissu tricoté selon la revendication 2, dans lequel le fil de fibres discontinues est un fil cellulosique.

4. Un tissu tricoté selon l'une quelconque des revendications 1 à 3, dans lequel le fil contractile comprend un élasthanne, ou bien nu ou bien recouvert d'un deuxième fil.

5. Un tissu tricoté selon la revendication 4, dans lequel l'élasthanne a une finesse comprise entre 33 et 156 dtex.

6. Un tissu tricoté selon l'une quelconque des revendications précédentes, dans lequel le monofil a une finesse comprise entre 10 et 45 dtex.

7. Un tissu tricoté selon la revendication 4 ou la revendication 5, dans lequel l'élasthanne est recouvert d'un polyamide ayant une finesse comprise entre 33 et 78 dtex.

8. Un tissu tricoté delon l'une quelconque des revendications 1 à 7 comprenant une base du monofil de polyamide et d'élasthanne recouvert d'un polyamide et un dessin de coton de fibres discontinues.

9. Un procédé de fabrication d'un tissu tricoté extensible ayant l'aspect de la dentelle, caractérisé par le tricotage d'un filament synthétique monofilaire ensemble avec un fil contractile pour former une base et un troisième fil pour former un dessin ayant l'aspect de dentelle et par le thermofixage du tissu tricoté à un température entre 185 et 205°C.
